

Feb. 13, 1934.

H. SCOTT

1,947,065

BIMETAL THERMOSTAT

Filed April 23, 1930



WITNESSES.

*E. A. McElroy*  
*H. M. Buehler*

INVENTOR

*Howard Scott*

BY  
*Wesley J. Carr*  
ATTORNEY

## UNITED STATES PATENT OFFICE

1,947,065

## BIMETAL THERMOSTAT

Howard Scott, Wilkinsburg, Pa., assignor to  
Westinghouse Electric & Manufacturing Company, a corporation of Pennsylvania

Application April 23, 1930. Serial No. 446,779

5 Claims. (Cl. 297—15)

My invention relates to thermally actuatable devices and particularly to bi-metallic thermostats.

The main object of my invention is to provide a bi-metallic thermostat which shall have improved fabricating properties, relatively high deflection for a predetermined temperature change and which shall retain its inherent strength up to a relatively high temperature.

Another object of my invention is to provide a highly efficient bi-metal thermostat that shall be adapted for use in the control of relatively low temperature values while maintaining all of the desirable characteristics as to strength and deflection.

In practicing my invention, I provide a high-expansion component including major and substantially equal portions of copper, nickel and zinc and with or without admixtures of minor portions of aluminum and manganese. The low-expansion component of the combination is a ferrous alloy containing a major portion of iron, a minor portion of nickel and relatively small quantities of cobalt and manganese and a still smaller quantity of carbon.

The single figure of the drawing is a sectional view of a bi-metal bar embodying my invention.

When brass is used as the high-expansion component of a bi-metal thermostat, the temperature range over which a combination including a high-expansion component of brass may be used is relatively limited. The fabricating characteristics of a bi-metal element of the kind having a copper base component leave much to be desired. The high-expansion component in this case, is

softer, and it is highly desirable that its hardness characteristic be increased and, in the case of copper-base alloys, this requires the introduction of constituent or metal which will not materially decrease the solid solubility of zinc. I have found that nickel accomplishes this function very effectively and, at the same time, materially increases the high-temperature strength of the component over that of the basic copper-zinc alloys. Aluminum and manganese may also be added with substantial benefits to the strength of the component at high temperatures. Aluminum may be considered as a substitute for zinc, and manganese may be considered as a substitute for copper.

When a brass-base alloy is combined with a ferrous alloy to constitute a bi-metallic thermostat, the problem of similar hardness values of the two components may have to be considered. It is, of course, obvious that it is highly desirable to have the hardness of the two bi-metal com-

ponents substantially the same, in order that both components may respond in substantially the same degree, to the rolling and other fabricating processes. It may be necessary to adjust the amount of beta constituent in the brass by a control in regard to the amount of zinc and of aluminum for a given relation of copper to nickel to manganese, in order that substantially the same range of hardness changes may be obtained in the high expansion component, during the cold-rolling process, as exists in the low-expansion component.

I have illustrated a bi-metal bar including a high-expansion member 11 and a low-expansion member 12 suitably united, as by welding, each member being of the composition hereinafter set forth.

A representative list of percentages of the various metals which I prefer to utilize in my improved high-expansion component is given below:

*High expansion component*

| No. | %Cu   | %Ni   | %Zn   | %Al | %Mn |
|-----|-------|-------|-------|-----|-----|
| 1   | 25-60 | 20-40 | 20-35 | 0   | 0   |
| 2   | 41.0  | 37.9  | 21.1  | 0   | 0   |
| 3   | 50.6  | 23.4  | 26.0  | 0   | 0   |
| 4   | 33.9  | 31.3  | 34.8  | 0   | 0   |
| 5   | 31.0  | 29.0  | 30.0  | 0   | 10  |
| 6   | 35.0  | 32.0  | 30.0  | 3   | 0   |
| 7   | 32.0  | 29.0  | 30.0  | 2   | 7   |

A table of preferred compositions of the low-expansion component of my improved bimetal thermostat is given below.

*Low expansion component*

| No. | %Ni   | %Co  | %Mn     | %C    | Remainder   |
|-----|-------|------|---------|-------|-------------|
| 1   | 35-39 | <2.0 | 0.2-0.5 | 0-0.3 | Fe + impur. |
| 2   | 36.0  | <2.0 | 0.3     | 0.1   | " "         |
| 3   | 27-32 | 2-10 | 0.2-0.8 | 0-0.3 | " "         |
| 4   | 28.7  | 7.3  | 0.7     | 0.1   | " "         |
| 5   | 30.0  | 5.5  | 0.2     | 0.1   | " "         |

I have found that bi-metal thermostats, in which the cooperating component include one or another combination of alloys given above in the two tables have improved fabricating characteristics, particularly as to their having substantially the same degrees of hardness. I have found also that bi-metal thermostats made of alloys of this kind will have a higher temperature range in the low-temperature field without loss of sensitivity or deflection than the bi-metallic thermostats which have been in use heretofore and

which utilized, as their high-expansion component a plain brass, or pure copper-zinc alloy.

Various modifications may be made in the device embodying my invention and I desire, therefore, that only such limitations shall be placed thereon as are set forth in the appended claims.

I claim as my invention:

- 10 1. A thermostatic element comprising a pair of cooperating metallic members having different temperature coefficients of expansion, the member having the higher temperature coefficient of expansion being an alloy including from 20% to 40% nickel, 60% to 25% copper and 20% to 35% zinc and the member having the lower temperature coefficient of expansion being an iron alloy including from 30% to 39% nickel, from 2% to 10% cobalt and traces of manganese and carbon.
- 15 2. A thermostatic element comprising a pair of cooperating metallic members having different temperature coefficients of expansion, the high-expansion member including substantially thirty to thirty three and one third per cent each of copper, nickel and zinc and the low-expansion member consisting of substantially thirty three per cent nickel, between two and ten per cent cobalt, traces of carbon and manganese, the remainder being iron.
- 20 3. A thermostatic element comprising a pair of metallic members having different temperature coefficients of expansion, the member having the higher temperature coefficient of expansion being

an alloy including substantially thirty to thirty-three and one-third per cent each of nickel, copper and zinc, and the member having the lower temperature coefficient of expansion being an alloy including between twenty-seven per cent and thirty-two per cent of nickel, between two per cent and ten per cent of cobalt, between two tenths and eight tenths per cent of manganese, between one tenth and three tenths per cent of carbon, the remainder being iron.

4. A thermostatic element comprising a pair of cooperating metallic members having different temperature coefficients of expansion, the high-expansion member consisting of substantially thirty-three per cent each of copper and of nickel, slightly less than thirty-three per cent of zinc, the remainder being aluminum, the low-expansion member including slightly less than thirty-three per cent of nickel, two per cent to ten per cent of cobalt, traces of each of manganese and carbon, the remainder being iron.

5. A thermostatic element comprising a pair of cooperating metallic members having different temperature coefficients of expansion, the high-expansion member consisting of substantially thirty per cent each of copper, nickel and zinc, the remainder being manganese, the low-expansion member consisting of substantially thirty-three per cent nickel, from two to ten per cent cobalt, between two tenths and eight tenths of one per cent of manganese and a trace of carbon, the remainder being iron.

HOWARD SCOTT.

36

110

40

115

45

120

50

125

55

130

60

135

65

140

70

145

75

150